

# UNITED STATES PATENT OFFICE.

WILLIAM N. BLAKEMAN, JR., OF MOUNT VERNON, NEW YORK.

## PAINT COMPOSITION.

1,423,390.

Specification of Letters Patent. Patented July 18, 1922.

No Drawing.

Application filed October 5, 1921. Serial No. 505,624.

To all whom it may concern:

Be it known that I, WILLIAM N. BLAKEMAN, Jr., a citizen of the United States, and resident of the city of Mount Vernon, in the county of Westchester and State of New York, have invented a new and useful Paint Composition, which invention is fully set forth in the following specification.

The object of this invention is to produce 10 a paint-composition which will show an increased resistance to weathering attacks and form a more permanent covering than the compositions now in use.

The present system of structural painting 15 is largely based upon the unique union of Dutch white lead as a pigment and linseed oil as a vehicle. These, when properly ground together, form a hydrated metallic soap, which, when spread on a plain surface, furnishes a smooth and homogeneous 20 insoluble film. The atmospheric elements, however, soon attack the bond, which is the oil vehicle, in this combination, and cause it to pass by insensible gradations from an 25 insoluble to a soluble condition, relaxing the bonding effect, releasing the pigment, and thus rapidly disintegrating the paint. This early destruction of the present paint films, by atmospheric hydrolysis, aided by a weak 30 alkaline reaction of the Dutch white lead pigment, is owing to the yielding character of linseed oil to weak hydrolytic influences; as, being strong in its oxygen affinities, it is 35 feeble in its resistance to even weak atmospheric hydrolytic action, becoming progressively sensitive to incipient hydrolysis by its progressive oxidation.

I have discovered that this disintegration 40 of all such oil-paint films can be delayed very greatly in its inception, and its progressive development indefinitely retarded, by reinforcing and fortifying the oil-vehicle with non-drying oils or fats showing a resistance to feeble saponifying attack or a repellent 45 indifference to incipient atmospheric hydrolysis, so that, such non-drying oils or fats will enter into combination with any drying-oil-vehicle, or drying-oil paint-compound.

50 The non-drying oils or fats which may be used are those belonging to the group of vegetable fatty oils, and of these, I prefer cocoanut oil and palm-kernel oil (or palm nut oil) both of which have a high resistance to weak hydrolytic action. These substances, which are flowing oils at summer

heats, but chill to a solid or semi-solid condition at somewhat lower temperatures, are miscible with and soluble in oil vehicles by the aid of heat and can be introduced to 60 the extent of from 5% to 20%, and will not cloud, flock, or chill out, but will remain in clear solution at temperatures very much below their thickening point. The result will be a great improvement in the spreading power of the vehicle for all pigments, particularly anhydrous pigments, and an increased resistance of the paint to atmospheric and abrasive influences. 65

Because of its abundance on the market, 70 I prefer to use cocoanut oil, and if five or six parts of linseed oil, carrying 10% of cocoanut oil, be ground with twelve parts of Dutch white lead, and spread on a plain surface, the mixture will firm to the touch 75 in eight or nine hours, under favorable atmospheric conditions, and subsequently indurate into a durable film, the resistance of the film to the elements being strongly supported by the presence of the cocoanut oil, 80 and the life of the paint greatly prolonged.

I have further discovered, that tung oil 85 is a very efficient solvent for these non-drying oils and fats even at common temperatures, when they are in a solid or semi-solid condition, and, when added in the proportion of from 12% to 15% to the oil-vehicle, prevents clouding or flocking at temperatures approaching freezing, and reduces the firming of the paint to one-third or one-half 90 the time—thus: If five or six parts of linseed oil, carrying 10% of cocoanut oil and 15% of tung oil, be ground with twelve parts of Dutch white lead, and spread on a plain surface, the mixture will firm to the touch in 95 from two and one-half to three hours, under favorable atmospheric conditions, and subsequently indurate into a permanent film resistant to atmospheric and abrasive influence. A mixture of six parts of cotton-seed 100 oil carrying 15% of tung oil and 10% of cocoanut oil, and ten parts of zinc-lead (composed of 60% zinc oxide and 40% lead sulphate) will firm to the touch in four or five hours under like atmospheric conditions. 105

Very satisfactory compositions can be formed, especially with anhydrous pigments, by using in the vehicle a proportion of a mineral oil of the Texas type, either in an untreated condition, or hydrogenated 110 or oxidized or both; or a mineral oil of the Pennsylvania type, hydrogenated or oxi-

dized, or both. I prefer oxidized Texas oil. Thus, if six parts of cottonseed oil, carrying 5% of cocoanut oil, 15% of tung oil and 10% of oxidized Texas oil, be ground with 5 ten parts of zinc-lead, the mixture, when spread, will firm and indurate satisfactorily and form an economical and permanent paint.

With slight changes in proportions of 10 vehicles and pigments, all the oils (drying, semi-drying, non-drying, and mineral) and all the pigments (hydrated and anhydrous) which fall within the economical scope of the painting art, can be employed. The 15 proportions of the various factors in the composition, will be governed by the character of the pigments and vehicles used, and the results desired.

In all cases, the usual proportion of a suitable commercial drier is to be used.

It will, of course, be understood that by the term "oil," as used in this specification and in the claims, to designate the vegetable oils and fats which have a high resistance to 25 hydrolysis, I intend to cover the use of such substances, whether they are in liquid, semi-solid, or solid, condition at the time of use.

The mixture of non-drying vegetable fatty oils having a high resistance to hydrolysis, with other fatty oils, is broadly 30 claimed in my application No. 505626 filed herewith; the use of such non-drying oils in paint-vehicles is specifically claimed in application No. 461,961, filed April 16, 1921; 35 and the grinding of pigments, to paste form,

in such non-drying oils, is specifically claimed in application No. 505625 filed herewith.

Having thus fully described my invention, I claim:

1. A paint-composition, carrying a proportion of non-drying vegetable fatty oil of high resistance to hydrolysis.

2. A paint-composition carrying a proportion of cocoanut oil.

3. A paint-composition carrying a proportion of non-drying vegetable fatty oil of high resistance to hydrolysis, and tung oil.

4. A paint-composition carrying a proportion of cocoanut oil and tung oil.

5. A paint-composition comprising a fatty oil; a pigment; and a non-drying vegetable fatty oil of high resistance to hydrolysis.

6. A paint-composition comprising a fatty oil; a pigment; and cocoanut oil.

7. A paint-composition comprising a fatty oil; a pigment; a non-drying vegetable fatty oil of high resistance to hydrolysis; and tung oil.

8. A paint-composition comprising a fatty oil; a pigment; cocoanut oil; and tung oil.

9. A paint-composition comprising a fatty oil; a pigment; a non-drying vegetable fatty oil of high resistance to hydrolysis; tung oil; and a mineral oil.

10. A paint-composition comprising a fatty oil; a pigment; cocoanut oil; tung oil; and a mineral oil.

WM. N. BLAKEMAN, JR.